

June 5, 1928.

1,672,432

G. W. SPALDING

GARMENT AND METHOD OF MAKING SAME

Filed Sept. 21, 1927

Fig. 1.



Fig. 2.



Inventors:

George W. Spalding,  
by *Charles F. Edwards*,  
J. M. G.

Patented June 5, 1928.

1,672,432

## UNITED STATES PATENT OFFICE.

GEORGE WANTON SPALDING, OF WORCESTER, MASSACHUSETTS, ASSIGNOR TO THE ROYAL WORCESTER CORSET COMPANY, A CORPORATION OF MASSACHUSETTS.

### GARMENT AND METHOD OF MAKING SAME.

Application filed September 21, 1927. Serial No. 221,004.

In stitching in sections or gores of elastic fabrics, comprising rubber threads or strands, in making various garments, said rubber threads or strands are often pierced 5 by the needles of the sewing machines so that they are cut through or weakened, thereby becoming easily broken, when the garment is stretched or under tension. These cut or broken strands are liable to draw out 10 when the garment is under tension, thereby rendering the garment more or less imperfect or unsightly.

The present invention has for its object to avoid this objection, and this result is arrived at by vulcanizing the edges of the elastic sections or gores to be stitched, before they are sewed into the garments. When the edges of elastic gores or sections have been thus vulcanized the rubber threads or 20 strands are caused to adhere to the textile cotton or silk threads or yarns of the fabric, thus making the vulcanized edges practically homogeneous, so that if the rubber threads are pierced or cut by the needles of 25 the sewing machines in making up the garments these rubber threads are so anchored or fastened in that they cannot pull out even when cut or broken.

In carrying the invention into effect the 30 edges of the elastic fabrics which are to be stitched into garments, and which contain rubber threads or strands, are preferably fed through a guide or holder to which is also fed a rubber cement. The sections or gores 35 of elastic fabrics thus treated are then subjected, for about fifteen minutes, to the action of heat at a temperature of about 240° F., thus vulcanizing the edges of the elastic fabrics so that the rubber threads or strands 40 in said fabrics are caused to adhere to the textile threads or yarns of the fabrics, and are thus anchored in place so that, even if cut or broken, they cannot pull out.

In the accompanying drawing Fig. 1 is a broken-out section of a girdle embodying 45 the invention, and Fig. 2 is a detail view of one of the elastic gores or sections having vulcanized edges.

Referring to the drawing, 12 denotes sections or gores of elastic fabric comprising 50 rubber threads or strands, and 13 denotes the non-elastic sections of the garment, which may be provided with stocking holders the straps 14 of which are broken away for simplicity of illustration. In other words, 55 the girdle shown is of usual construction excepting as to the embodiment of the present invention. The edges 15 of the elastic sections or gores 12 have been treated and vulcanized by the means hereinbefore set forth, and when stitched-in these vulcanized edges are wholly or partially covered by the 60 textile non-elastic sections of the garment.

While the invention is herein illustrated as being applied to a girdle, it will be understood that said invention may be embodied in other garments, such as corsets, corselets, brassières, bandeaux, step-ins and other compressing or confining garments comprising sections of elastic fabrics having 65 rubber threads or strands.

Having thus described my invention I claim and desire to secure by Letters Patent:

A garment comprising stitched-in sections 70 of elastic fabric the edges of which contain a rubber cement, said sections comprising 75 rubber threads, and said edges with the rubber cement therein being vulcanized to anchor the rubber threads at said edges, the stitches passing through said vulcanized 80 edges and the body of the garment.

In testimony whereof I affix my signature.

GEORGE WANTON SPALDING.